

## UNITED STATES PATENT OFFICE

2,478,396

ACTIVATION OF CELLULOSE FOR  
ACYLATION

William B. Hincke, Kingsport, Tenn., and Carl J. Malm, Rochester, N. Y., assignors to Eastman Kodak Company, Rochester, N. Y., a corporation of New Jersey

No Drawing. Application June 27, 1945,  
Serial No. 601,918

5 Claims. (Cl. 260—225)

1

This invention relates to the activation of cellulose preparatory to acylation in which the cellulose in the form of a slurry in distilled or demineralized water free of added chemicals is boiled 2-4 hours and the water is removed by means of lower fatty acid.

Cellulose, particularly wood pulp cellulose, as normally obtained, even that classifiable as refined high cellulose material, contains a small amount of hornified amorphous material which is particularly resistant to acylation. Even though the cellulose is mechanically disintegrated or opened up to assure contacting of the acylating liquids with all the particles of cellulose it is still difficult to uniformly acylate cellulose containing hornified material with fatty acid anhydride and catalyst. Often a residual haze is found in the reaction mass resulting after acylation which can be removed only with great difficulty.

To facilitate the acylation of cellulose pretreatment with acetic acid has been resorted to. Glacial acetic acid, as normally employed in pretreatment operations, leaves much to be desired as a swelling agent for the horny material found in some cellulose, and the anhydrous fatty acids having more carbon atoms than acetic, such as propionic or butyric, are of much less value than acetic acid for facilitating the acylation reaction with fatty acid anhydride. The use of higher than normal amounts of catalyst, higher temperatures or longer times of reaction in the subsequent esterification step do not compensate for the poor pretreatment and result in more complete acylation of the cellulose but only in more breakdown or acetolysis of the cellulose in the final cellulose ester. Such intensified operations result in a cellulose ester having a viscosity too low for use in preparing commercial products.

One object of our invention is to provide a method of activating cellulose, particularly that having some horny, unreactive particles therein, to render it readily and uniformly reactive with lower fatty acid anhydride in ordinary cellulose acylation processes. Another object of our invention is to provide an effective method of activating cellulose requiring but a short time of treatment. A further object of our invention is to provide a method of activating cellulose, in which water acts as the activating agent yet the pretreated cellulose is obtained in the form of cellulose mixed with only a small proportion of lower fatty acid. Other objects of our invention will appear herein.

These objects of our invention are accomplished

5 by forming the cellulose into a slurry in low mineral content water, without the addition of chemicals thereto, boiling the slurry for 2 to 4 hours and then removing the water from the cellulose with lower fatty acid so that there results an activated cellulose moistened with the lower fatty acid.

Our pretreatment method may be applied to any cellulose, suitable for acylation purposes, 10 which can be slurried with water, an advantage being that only a short time of treatment is necessary. Our pretreatment method however is particularly adapted to cellulose which has a non-uniform nature because of the presence of horny, 15 amorphous particles distributed therethrough. For instance, acetylation grade wood pulp cellulose is supplied ordinarily in the form of rolls of dry sheets in which hard particles of cellulose are found distributed through the sheet.

20 The cellulose in accordance with our invention is mixed with or agitated in 15 to 25 parts of distilled or low mineral content water (per part of cellulose) to form a suspension or slurry of the cellulose fibers therein. The water used 25 is one which has a mineral content of less than 20 parts per million. This may be distilled water or a demineralized water. Obviously the lower the mineral content, the more suitable is the water for use in our activation process. The 30 term "low mineral content water" as used herein is to be understood as referring to water having a mineral content of 0-20 parts per million therein. The proportion of water employed is not critical being sufficient to give a good slurry and conducive to uniform boiling. At least 15 parts of 35 water is ordinarily necessary for this. The cellulose after suspending in water is subjected to boiling for from 2 to 4 hours and a highly activated cellulose results.

40 Before using this cellulose for esterification it is desirable to remove the water therefrom. It is a feature of our invention that the water is removed from the cellulose in such a manner that the product consists of highly reactive cellulose moistened by lower fatty acid. The water 45 may be directly removed from the cellulose with fatty acid, however, removal is best and most economically accomplished by first removing the bulk of the water from the cellulose by mechanical means such as by means of squeeze rolls, screw presses, suction filters, centrifuges or the like. To retain the swollen reactive condition of the cellulose the remaining 1-2 parts of water present therein is extracted or displaced with a lower fatty acid, either acetic, propionic or butyric

or their mixtures. This may be accomplished for instance by a counter current method or by subjecting the cellulose to suction while supplying acid thereto. If considerable acid remains on the cellulose it may be desirable to subject it to squeezing or other mechanical removal means before acylation. The acid damp cellulose obtained is suitable for charging directly to the acylation mixer for direct acylation with fatty acid anhydride and catalyst.

The activated cellulose obtained may be employed for making cellulose acetate or cellulose mixed esters in which acetic anhydride is employed as the esterifying agent or for making high propionyl or high butyryl cellulose esters. In making the latter at least a large proportion or even the entire anhydride may be propionic or butyric anhydride as the esterifying agent. As these anhydrides are more sluggish in acylating effect than acetic anhydride, it is important that the cellulose employed therein be highly reactive. Although ordinarily acetic acid will be employed to displace the water on the cellulose, in these cases where little or no acetyl is desired in the cellulose esterification mixture, butyric or propionic acid may be employed for this purpose.

The following examples illustrate our invention:

*Example I*

One part of wood cellulose sulfite pulp, having a high  $\alpha$ -cellulose content was slurried with 20 parts of demineralized water having a mineral content of approximately 10 parts per million and the mass was boiled for 3 hours in a jacketed tank. The slurry was centrifuged to a content of about 1 part of water per part of cellulose. While still in the rotating centrifuge, the wet cellulose mat was extracted by spraying onto it while the centrifuge was operating successive amounts of acetic acid of increasing concentration, such as was obtained by saving the effluent from previously dewatered batches. By so doing a counter current system is effected with a minimum use of final glacial dewatering acid. The first obtained, most dilute acid was sent to recovery to concentrate the same.

The acid wet cellulose was centrifuged down so as to contain 1 part of acid and 0.01 to 0.03 part of water per part of dry cellulose. This cellulose was then charged directly to an acylator containing 3 parts of acetic anhydride and .05 part of sulfuric acid catalyst and was acylated therein. The cellulose reacted rapidly to give a mass of high clarity showing the absence of unacylated particles therein.

*Example II*

The procedure of the preceding example was repeated except that butyric acid was employed to remove the water from the cellulose after the boiling and removal of the bulk of the water by centrifuging. The activated cellulose containing butyric acid was charged into an esterification mixer containing 4½ parts of butyric anhydride and .04 part of sulfuric acid catalyst and the cellulose was butyrylated, the temperature being controlled so that it did not exceed 90° F. over the entire reaction. The cellulose reacted readily to give a mass of high clarity.

*Example III*

One part of wood cellulose sulfite pulp of high alpha-cellulose content was slurried and boiled with 25 parts of demineralized water having a mineral content of approximately 10 parts per

million for 3 hours in a jacketed tank. This slurry was then thinned with more water so that the pulp could be formed into a web on a perforated stainless steel belt similar to that used on the wet end of a paper machine. This cellulose web on the perforated belt was then passed over suction boxes to remove the excess water and, following this, over a sequence of suction boxes where it was sprayed with acetic acid of increasing concentration in a counter current manner. From the last spray and suction box the cellulose mat was delivered substantially free from water and damp with 2-2½ parts of acetic acid. This mat was then charged to a continuous screw press to further remove the acetic acid to 1 part. The pressed mat was then broken up by passing it through a picker or hammer mill and charged to an acylation mixer containing 4½ parts of butyric anhydride and 0.05 part sulfuric acid catalyst. The cellulose reacted rapidly to a clear dope of cellulose acetate butyrate free from any unreacted cellulose particles.

*Example IV*

The cellulose boiling procedure of Example III was repeated except cotton linters were used. Following this butyric acid was used as the water extractant instead of acetic acid in passing the cellulose web over the counter current spray and suction box dewatering device. The cellulose mat delivered from the last suction box was damp with 2 parts butyric acid. This pulp was then charged without further centrifuging to an acylation mixer containing 4½ parts butyric anhydride and 0.05 part sulfuric acid catalyst. The ensuing reaction to a cellulose tributyrate was somewhat slower than to the mixed ester shown in Example III but the reaction was complete to an acid dope of high clarity.

*Example V*

The same pulping and boiling procedure was used as in Example III. However, in order to effect the countercurrent removal of water, an Oliver suction filter was used. This filter was equipped with a number of sprays so that acetic acid of increasing concentration could be passed through the cellulose mat in a countercurrent manner. After removal from the Oliver filter, the mat was passed through squeeze rolls where the acid was finally removed to 1 remaining part substantially free from water. This acetic acid damp cellulose was then charged to an acylation mixer as in Example III and a high butyryl mixed ester was prepared by rapidly reacting to a dope free from unacylated cellulose particles.

*Example VI*

One part of high alpha sulfite pulp was slurried in 25 parts of distilled water and the mass was boiled for 3 hours. The slurry was centrifuged to remove the bulk of the water and then dewatered by spraying acetic acid onto the centrifuging pulp mass until a cellulose was obtained having 1 part of acid and substantially no water (less than 0.02 part) per part of cellulose. The cellulose was picked apart and mixed with butyric anhydride and a little sulfuric acid catalyst in an acylation mixer cooled so that the temperature never exceeded 90° F. A cellulose ester of good quality was obtained.

When the term "substantially free of water" is used herein it is to be understood to mean less than 0.05 part of water and preferably less

than 0.03 part is present per part of dry cellulose.

We claim:

1. A method of activating cellulose containing a small amount of hornified amorphous material which is particularly resistant to acylation which consists in boiling a suspension of the cellulose in a large excess of water having a mineral content of less than 20 parts per million for two to four hours, subjecting the cellulose mass to pressure to remove water, at least one part of water remaining per part of cellulose and subsequently displacing the water in the cellulose with a fatty acid of 2-4 carbon atoms so as to give a cellulose containing fatty acid but substantially free of water therein.

2. A method of activating cellulose containing a small amount of hornified amorphous material which is particularly resistant to acylation which consists in boiling a suspension of the cellulose in a large excess of distilled water for two to four hours, subjecting the cellulose mass to pressure to remove water, at least one part of water remaining per part of cellulose and subsequently displacing the water in the cellulose with a fatty acid of 2-4 carbon atoms so as to give a cellulose containing fatty acid but substantially free of water therein.

3. A method of activating cellulose containing a small amount of hornified amorphous material which is particularly resistant to acylation which consists in boiling a suspension of the cellulose in a large excess of water having a mineral content of less than 20 parts per million for two to four hours, subjecting the cellulose mass to pressure to remove water, at least one part of water remaining per part of cellulose and subsequently displacing the water in the cellulose with acetic acid so as to give a cellulose containing acetic acid but substantially free of water. 40

4. A method of activating cellulose containing a small amount of hornified amorphous material which is particularly resistant to acylation which consists in boiling a suspension of the cellulose in a large excess of water having a mineral content of less than 20 parts per million for two to four hours, subjecting the cellulose to pressure to remove water, at least one part of water remaining per part of cellulose and subsequently displacing the water in the cellulose by a concurrent treatment thereof with acetic acid so as to give a cellulose containing acetic acid but substantially free of water therein.

5. A method of preparing cellulose acetate butyrate having a high butyryl content from a cellulose containing a small amount of hornified amorphous material which is resistant to acylation which consists in first boiling the cellulose in suspension in a large excess of low mineral content water, subjecting the cellulose to pressure to remove water, at least one part of water remaining per part of cellulose, displacing the water in the cellulose with acetic acid and then esterifying the cellulose with an esterification mixture comprising butyric anhydride and an acylation catalyst.

WILLIAM B. HINCKE.  
CARL J. MALM.

#### REFERENCES CITED

The following references are of record in the file of this patent:

#### UNITED STATES PATENTS

| 35 | Number    | Name          | Date          |
|----|-----------|---------------|---------------|
|    | 1,752,596 | Hubert et al. | Apr. 1, 1930  |
|    | 2,087,263 | Olsen         | July 20, 1937 |
|    | 2,112,115 | Richter       | Mar. 22, 1938 |
|    | 2,112,116 | Richter       | Mar. 22, 1938 |
|    | 2,152,071 | Malm          | Mar. 28, 1939 |